

## UNITED STATES PATENT OFFICE.

MARION F. NICHOLS, OF KNOXVILLE, TENNESSEE, ASSIGNOR OF ONE-HALF TO WILLIAM K. HUNTER, OF KNOXVILLE, TENNESSEE.

## PROCESS OF UNITING THE ENDS OF THREADS.

No Drawing.

Application filed November 17, 1925. Serial No. 69,707.

My invention relates to a method of cementing together the ends of spun yarn or thread, for producing a continuous thread free from knots, enlargements, or irregularities.

In the knitting of garments of various kinds, the spun yarn or thread passed to the needles, frequently contain knots, which cause the improper operation of the knitting machine, and the production of seconds or imperfect garments. In a large factory, the amount of seconds produced, is often considerable, with the result that heavy loss is incurred. The spun yards, or thread, frequently break when passing to the spools, or to the knitting machines, or prior to the sizing operation. When this occurs, it is the practice for the attendant to tie the ends of the broken yarn or thread together, and this produces the objectional knots.

As far as I am aware, no one has heretofore proposed to cement together the broken ends of spun yarn or thread which is passed to a knitting machine, for the purpose of eliminating the production of imperfect garments, due to the action of these knots upon the needles or other operating parts of the knitting machine.

In accordance with my invention, the ends of a broken, spun thread or yarn are secured together by a suitable cement, preferably a rapidly drying cement solution, in a manner that the break can hardly be detected. The union of these threads produces a joint which is not perceptively larger in diameter than the yarn or thread, and the joint is free from knots or irregularities, permitting the yarn or thread to pass smoothly through the needles of the knitting machine, thus obviating the flaws in the product and producing a perfect garment.

In the practice of my method, I take a cement solution, which will preferably dry rapidly, and apply the same to the ends of the spun yarn or thread to be united, and quickly bring these coated ends together in overlapping relation, and then subject them to a slight and rapid rolling or twisting operation, which may be by hand or machinery. In a few seconds, the ends of the yarn or thread are united more firmly than the orig-

inal thread, and the diameter of the joint is not perceptibly different from the diameter of the thread or yarn. If desired, the ends of the yarn or thread to be united may be partially frayed or tapered, and these tapered overlapping ends are thus cemented together. Instead of applying the cement to the ends before they are brought together, the cement may be applied afterwards and the same twisting and rolling action applied to such ends.

In the production of the rapidly drying cement solution, I make a solution of any cellulose material, such as gun cotton, pyroxylin, nitro-cellulose, or any of the derivatives of cellulose, in a suitable solvent, such as ether, or ether and alcohol, or acetone. This cement solution is applied to the ends of the spun yarn or thread, as stated. I have found that satisfactory results are obtained by employing a cellulose solution composed of substantially 30 grams of a soluble cellulose material, 750 cubic centimeters of ether, and 250 cubic centimeters of alcohol. This cement solution will dry rapidly, will securely unite the fibers in the spun yarn or thread, and is insoluble in water.

While the cement solution, above described, is one well adapted for the practice of my invention, yet the proportions of the ingredients may be somewhat varied, as may be found advantageous, for use upon different threads or yarns.

I have found that yarns or threads of cotton, wool, silk or linen, or other fibrous material, may be properly united by my cement solution.

It is to be understood that the form of my invention herein described is to be taken as a preferred example of the same, and that certain changes may be resorted to in the order of the steps of the method and that chemical equivalents may be employed in the cement composition, without departing from the spirit of my invention or the scope of the subjoined claims.

Having thus described my invention, I claim:

1. In a method of knitting, uniting the ends of spun strands by means of an adhesive in such a manner that knots or similar

enlargements are eliminated, and feeding the united spun strands to a knitting machine. union being effected in such a manner that knots or similar enlargements are eliminated, and feeding the united spun strands to a knitting machine.

2. In a method of knitting, uniting the ends of spun strands by overlapping such ends and twisting the same under suitable pressure in the presence of a highly volatile adhesive which is insoluble in water, the

In testimony whereof I affix my signature.

MARION F. NICHOLS.